

Patented June 11, 1940

2,203,670

# UNITED STATES PATENT OFFICE

2,203,670

## METHOD OF TREATING ELECTROLYTIC COATINGS ON MAGNESIUM AND ITS ALLOYS

Robert W. Buxford, Kensington, Md.

No Drawing. Application June 29, 1937,  
Serial No. 150,932

7 Claims. (CL 204—1)

(Granted under the act of March 3, 1883, as  
amended April 30, 1928; 370 O. G. 757)

This invention relates to the treatment of electrolytically formed coatings on magnesium and its alloys in which magnesium predominates and one of its objects is to increase the durability 5 and the protective characteristics of the film by sealing the coating.

The method specifically relates to the treating of electrolytic coatings on magnesium and its alloys with a solution in the presence of heat so 10 as to form a seal that not only increases the durability of the article coated to wear but also improves its resistance to corrosion.

The article to be treated in this manner, which has been coated electrolytically, is washed free 15 of solution, providing the electrolytic bath is basically different from the solution used in my sealing method and is then immersed in a hot solution of sealing compounds, preferably at or above the boiling point of the solution, but below 20 the fusion point of the metal.

The sealing solution should contain a corrosion 25 inhibiting ion such as either a chromate or dichromate and a second water soluble salt containing an ion of either manganese or chromium or borate, phosphate, fluoride or a combination of any of the said second salts. The concentration of the salts is limited only by their solubility, but may be varied to conform with time of application and quality of seal. Good seals of 30 coated metal have been obtained by subjecting the coatings to treatment for periods varying from five minutes to one hour.

Specifically, as an example, if an anodic coating 35 be formed on magnesium or its alloys in a bath of 10 percent dichromate and a 2 per cent monobasic phosphate and the coating has been washed free of anodizing solution, its corrosion resistance will be greatly improved if it is immersed in a solution of dichromate and manganese sulphate at boiling temperature of water 40 or above. The sealing solution may be varied to contain a trivalent chromium salt as chromium acetate or sulphate or fluoride. A chromate may be introduced or substituted in the solution or a phosphate may be substituted or added when the 45 solution is of such composition not to cause detrimental inter-solution reactions.

It should be understood that the protection 50 obtained by my treatment is dependent on the presence of an electrolytic coating and is not a prime surface treatment.

In the sealing treatment herein set forth a 55 chemical reaction is produced improving the characteristics of the electrolytic coating. This change is evinced by a corrosion test wherein two identical anodized articles, one sealed by my method and one unsealed, disclosed over a corrosion period that the sealed coating did not change in color, whereas the unsealed coating 60 showed a radical change in color.

As further examples of compositions which will satisfactorily seal electrolytic coatings on magnesium, the following are cited:

|                            | Per Cent   |
|----------------------------|------------|
| (a) Dichromate             | 1 to 30    |
| Chromium fluoride          | 25 to 10   |
| (b) Sodium dichromate      | 10         |
| Chromium fluoride          | 1          |
| (c) Sodium dichromate      | 10         |
| Monobasic sodium phosphate | 10         |
| Chromium fluoride          | 1          |
| (d) Sodium dichromate      | 10         |
| Zinc phosphate             | 1 15       |
| Magnesium phosphate        | 1          |
| Chromium fluoride          | 1          |
| (e) Sodium dichromate      | 10         |
| Sodium phosphate           | 10         |
| Chromium sulphate          | 1 20       |
| (f) Dichromate             | 1 to 30    |
| Borate                     | 1 to 30    |
| (g) Sodium dichromate      | 10         |
| Sodium borate              | 5 25       |
| (h) Dichromate             | 1 to 30    |
| Sulphate                   | 1 to 30    |
| (i) Dichromate             | 10         |
| Manganous sulphate         | 10 30      |
| (j) Ammonium dichromate    | 10 to 20   |
| Manganous sulphate         | 5 to 10    |
| (k) Zinc chromate          | 1 35       |
| Manganous sulphate         | 1          |
| Chromium fluoride          | 1          |
| (l) Ammonium dichromate    | 5 to 10    |
| Sodium borate              | 5 to 10    |
| Manganous sulphate         | 5 to 10 40 |
| (m) Dichromate             | 1 to 30    |
| Fluoride                   | 25 to 20   |
| (n) Dichromate             | 10         |
| Sodium fluoride            | 5 45       |
| Chromium fluoride          | 1          |
| (o) Dichromate             | 1 to 30    |
| Phosphate                  | 1 to 30    |
|                            | 50         |
| (p) Sodium phosphate       | 10         |
| Dichromate                 | 10         |
| Chromium fluoride          | 1          |
| (q) Dichromate             | 10         |
| Manganous sulphate         | 10 55      |
| Zinc phosphate             | 1          |
| (r) Zinc chromate          | 1          |
| Sodium dichromate          | 5          |
| Chromium fluoride          | 1 60       |

6 A double dip may also be used such as first immersing the electrolytically coated article in a solution of dichromate and phosphates followed by an immersion in a solution of manganese and chromium sulphate. Ammonium and other salts may be substituted for the sodium and potassium salts.

10 The above mentioned substances used in the magnesium treatments are mentioned by way of illustration and not by limitation, since the invention comprehends treatments of the character indicated broadly above and is not to be limited except by the appended claims.

15 The invention described herein may be manufactured used by or for the Government of the United States of America for governmental purposes without the payment of any royalties thereon or therefor.

What I claim is:

20 1. The method of producing corrosion resistant coatings on magnesium or magnesium alloys in which magnesium predominates comprising forming on the metal an anodic coating produced by reaction with magnesium and subjecting the 25 coating to a non-electrolytic treatment for five minutes to one hour in an aqueous solution containing 1 to 30 percent water soluble dichromate and 8 to 12 percent manganese sulphate, and maintaining the temperature of the solution during treatment substantially equivalent to the 30 boiling point of the solution.

35 2. The method of producing corrosion resistant coatings on magnesium or magnesium alloys in which magnesium predominates comprising forming on the metal an anodic coating produced by reaction with magnesium and subjecting the 40 coating to a non-electrolytic treatment from five to sixty minutes in an aqueous solution containing 8 to 12 percent water soluble dichromate and 8 to 12 percent water soluble sodium phosphate, and maintaining the temperature of the solution during treatment substantially equivalent to the 45 boiling point of the solution.

45 3. The method of producing corrosion resistant 50 coatings on magnesium or alloys thereof in which magnesium predominates comprising forming on the metal an anodic coating produced by reaction with magnesium, and subjecting said coating to a non-electrolytic treatment in an aqueous solution containing manganese sulphate and a water-sol-

uble compound selected from the group consisting of the chromates and dichromates, the pH of such solution being on the acid side.

5 4. The method of producing corrosion resistant coatings on magnesium or alloys thereof in which magnesium predominates comprising forming on the metal an anodic coating produced by reaction with magnesium, and subjecting said coating to a non-electrolytic treatment in an aqueous solution containing at least 1 per cent of a water-soluble sulphate and of a water-soluble compound selected from the group consisting of the chromates and dichromates, the pH of such solution being on the acid side.

10 5. The method of producing corrosion resistant 15 coatings on magnesium or alloys thereof in which magnesium predominates comprising forming on the metal an anodic coating produced by reaction with magnesium, and subjecting said coating to a non-electrolytic treatment in an aqueous solution containing a water-soluble phosphate and a water-soluble compound selected from the group consisting of the chromates and dichromates, the pH of such solution being on the acid side.

20 6. The method of producing corrosion resistant 25 coatings on magnesium or alloys thereof in which magnesium predominates comprising forming on the metal an anodic coating produced by reaction with magnesium, and subjecting said coating to a non-electrolytic treatment in an aqueous solution containing a water-soluble fluoride and a water-soluble compound selected from the group consisting of the chromates and dichromates, the pH of such solution being on the acid 30 side.

35 7. The method of producing corrosion resistant 40 coatings on magnesium or alloys thereof in which magnesium predominates comprising forming on the metal an anodic coating produced by reaction with magnesium, and subjecting said coating to a non-electrolytic treatment in an aqueous solution containing a water-soluble phosphate and a water-soluble compound selected from the group consisting of the chromates and dichromates, followed by a second non-electrolytic treatment in a solution containing manganese 45 sulphate and chromium sulphate.

ROBERT W. BUZZARD. 50